

April 30, 1935.

C. E. ROZEMA

1,999,259

METHOD OF MAKING AND FINISHING A WOOD PANEL

Filed July 24, 1933



*Inventor:*  
Charles E. Rozema,  
*By* Wm F. Freundreich,  
*Attest*

**Patented Apr. 30, 1935**

**1,999,259**

# UNITED STATES PATENT OFFICE

**1,999,259**

## **METHOD OF MAKING AND FINISHING A WOOD PANEL**

Charles E. Rozema, Grand Rapids, Mich., as signor, by mesne assignments, to Reconstruction Finance Corporation, a Federal corporation

Application July 24, 1933, Serial No. 681,898

**8 Claims. (Cl. 144—309)**

The present invention has for its object to make one or both faces of a plywood water-resistant and capable of withstanding attacks of other agencies through which wood is frequently damaged and, at the same time, give to the wood a fine surface finish without having to resort to the usual sanding operation or other similar expedients now commonly employed to produce a smooth surface.

10 Viewed in one of its aspects the present invention may be regarded as having for its object to treat wood in a simple and novel manner so that it is protected as fully as though it had thereon several coats of good paint without the presence, however, of any superficial coating which may be scraped off in the manner of paint.

15

In carrying out my invention I impregnate the wood surface with a fusible synthetic resin, preferably of the thermosetting type. This I accomplish by bringing the panel into a suitable condition as to temperature and moisture content, depositing the resin upon a face thereof and then applying a smoothing pressure, preferably by running a roller over the resin-coated face of the panel. The heat in the wood causes the resin to melt and, under the pressure of the roller, to flow into the wood to a depth of a few thousandths of an inch; giving a thorough impregnation of the surface fibers and filling the spaces between these fibers to form a continuous layer or film that does not project above the free surfaces of the surface fibers. While the layer or film of resin does not lie on top of the wood as would a layer of paint, yet it comes up to that surface and provides it with a characteristic gloss.

The resin may be colored, anilin dyes being conveniently employed for interior uses and light-fast pigments for faces to be exposed to the weather. It is not necessary to use colors that are ordinarily insoluble in water because, when water-soluble colors are mixed with the resin and fused into the wood, they become insoluble, probably because of a resin coating.

In order that the surface impregnation of a plywood panel be accomplished at a sufficiently slow cost, it must be carried out at the end of the operation of gluing the panel by the hot process. In gluing up panels with synthetic thermosetting resin as the adhesive, the panels on leaving the press are in appropriate condition for my treatment, because they will have such high temperature and such low moisture content that synthetic resins can be found with

1,999,259

# PATENT OFFICE

259

## MAKING AND FINISHING A PANEL

and Rapides, Mich., assignments, to Reconstruction, a Federal corpora-

333, Serial No. 681,898

which to carry out my process. If the gluing is done with blood albumen glue, the tempera-

ture may not be high enough, and it may be necessary to raise the temperature of the panels in the press beyond that required for the setting of the glue.

Therefore, viewed in one of its aspects, the present invention may be said to have for its object a simple and novel method of producing plywood and giving it a finished surface requiring no sanding, and being superficially impregnated with an inert weather-resisting synthetic resin that may be colored in whole or in part.

The various features of novelty whereby my invention is characterized will hereinafter be pointed out with particularity in the claims; but, for a full understanding of my invention and of its objects and advantages, reference may be had to the following detailed description taken in connection with the accompanying drawing, 2 wherein:

Figure 1 illustrates the gluing up of a multiple-ply panel between hot plates or cauls; Fig. 2 is a plan view of a fragment of the glued panel, showing synthetic resin overlying a face of the panel, 2 with the layer of resin being broken away at one corner; Fig. 3 is a section, on an enlarged scale, through a fragment of the panel, illustrating the rolling of the resin-coated face; and Fig. 4 is a view of the panel similar to that shown in Fig. 3, 3 at the end of the rolling operation.

Referring to the drawing, 1 represents a plywood panel or board which, in Fig. 1, is being glued in a hot press between hot plates or platens A and B. At the end of the gluing operation the panel contains very little moisture and has a high temperature. The moisture content of the panel upon removal from the press depends very much upon the temperature of the panel and the length of time that this temperature has been maintained; the temperature depending on the character of the glue and being such as to produce setting of the latter. Gluing temperature may in some instances be as low as 200° F. and in others, it may be 300° F. or more. For the higher

temperatures the moisture content is likely to be as low as two or three percent, whereas for the low temperature the moisture content may be considerably higher. Immediately after removal from the press and while the panel is in this hot, dry condition, a layer 2 of dry, comminuted synthetic resin, inert to weathering and preferably thermosetting, is deposited on a face of the panel. The heat of the panel melts the resin which flows into the dry wood. Pressure preferably is ap-

plied in a manner to force or aid in forcing the melted resin into the wood, conveniently through a roller C that is run over the coated face of the panel. The roller is preferably chilled so as to aid in quickly hardening the resin after it has entered the wood. It should be noted that the resin descends in the wood, forming a continuous protecting film reaching from the surface of the wood into the interior for a few thousandths of an inch, depending upon various factors such as the temperature of the panel, the quantity of resin, the temperature at which the resin melts, the kind of wood, and the pressure of the roller. For example, some films that I have measured have had a thickness no greater than five one-thousandths of an inch while others have had a thickness of twenty one-thousandths of an inch. In Figs. 3 and 4, which illustrate fragments of a panel on a greatly magnified scale, the dotted or stippled areas or zones 3 represent the zones permeated by the resin.

The resin may be colored, or the resin applied to certain areas of a panel may be colored and that over remaining areas of the face of the panel be left uncolored. Furthermore, where coloring is used, there may be a plurality of different colors. For example, the resin may be so colored and be laid down in such a manner as to produce stripes; there being shown in Fig. 2 a stripe 4 of one color and a stripe 5 of another color. Where the resin is to be uniformly distributed, the color may be applied to the panel first, if desired; insoluble colors being applied dry or suspended in a liquid medium to permit them to be applied by brushing, spraying or dipping. When the resin itself is colored, the coloring matter does not pass down into the wood to the same depth as does the resin, but does enter the wood to a sufficient depth to prevent its removal in the event that paint, varnish or other surface finish coatings are subsequently removed by the usual mechanical methods. Obviously, any desired decorative color scheme is possible. For example, instead of a striped effect, the appearance of burnt wood may be created.

The finishing process must be carried out promptly after the removal of the panels from the press, in order to avoid cooling to a temperature too low to melt the resin for the protecting film and to avoid the taking up of too much moisture from the surrounding air. This can be accomplished by carrying each panel directly from the press to a position under a shaking screen and thus causing it quickly to be uniformly covered with powdered resin and then immediately running it between pressure rollers. Handled in this way, it is evident that the cost of providing a panel with the protecting film of resin, over the cost of the resin itself, is not great, so that my improved plywood panels are not much more expensive than ordinary plywood panels.

It will, of course, be evident that any wood panel, whether multiple-ply or not, may be treated to provide it with the continuous protective film of resin, although at a higher cost if it must be heated and dried for that purpose alone. The final product, whether the surface-impregnating treatment be given to a panel that must first be heated and dried, or to a panel that comes from the gluing press hot and dry, has a surface inert to weathering, water-resistant to a high degree, and adapted to receive a good paint finish with a minimum amount of painting. Furthermore, the process in both cases eliminates the need of costly solvents for the resin and the fire hazard that

accompanies the use of such solvents, permits the use of resinous materials not readily mixed with solvents or else generally insoluble in solvents. In both cases the actual completion of the surfacing of the wood is very rapid when compared with the time that is required by varnishes and the like to dry, where the corresponding surface finish is produced by a varnish or paint coat.

While I have illustrated and described my improved process and product with particularity, I do not desire to be limited to all of the details thus illustrated and described; but intend to cover all methods and products thereof that come within the definitions constituting the appended claims.

I claim:

1. The method of treating a member of wood which consists in heating and drying it until it has a moisture content of only a very few percent and a high temperature, depositing on the face of said member while the latter is dry and hot a synthetic resin, and rolling the resin into the wood and causing all of it to penetrate below the plane of said face.

2. The method of treating a member of wood which consists in heating and drying it until it has a low moisture content and a high temperature, depositing on the face of said member while the latter is dry and hot a thermosetting synthetic resin, and pressing and cooling the resin to cause the latter to penetrate into the wood below the plane of said face.

3. The method of treating a member of wood which consists in heating and drying it until it has a low moisture content and a temperature of about 250° F. or more, depositing on the face of said member while the latter is still hot dry, powdered synthetic resin of a kind that is melted by the heat of said member, and pressing the resin into the hot wood.

4. The method of treating a member of wood which consists in heating and drying it until it has a low moisture content and a temperature of about 250° F. or more, depositing on the face of said member while the latter is still hot a powdered thermosetting synthetic resin of a kind that is melted by the heat of said member, and pressing the resin into the hot wood and simultaneously chilling it.

5. The method of producing and finishing a plywood panel which consists in gluing up a panel by a hot process, employing pieces of wood and glue of such moisture contents and applying heat to such a degree that the glued panel has a low moisture content and a high temperature upon leaving the press, and then, while the panel remains dry and hot, depositing on a face thereof a powdered synthetic resin that is melted by the heat of the panel, and applying pressure to squeeze the melted resin into the wood.

6. The method of producing and finishing a plywood panel which consists in gluing up a panel by a hot process, employing pieces of wood and glue of such moisture contents and applying heat to such a degree that the glued panel has a low moisture content and a high temperature upon leaving the press, and then, while the panel remains dry and hot, depositing on a face thereof a powdered thermosetting synthetic resin that is melted by the heat of the panel, and then pressing the resin into the hot wood and simultaneously chilling it.

7. The method of treating a member of wood which consists in heating and drying it until it

has a low moisture content and a high temperature, depositing on the face of said member while the latter is dry and hot a resinous material, and pressing the resin against the hot wood.

5. The method of treating a member of wood which consists in heating and drying it until it has a low moisture content and a high tempera-

ture, depositing on the face of said member while the latter is dry and hot a material that will not penetrate the wood at ordinary temperatures and melts at said high temperature, and pressing said material against the hot wood.

5

CHARLES E. ROZEMA.